

3,370,912  
**PROCESS OF SIMULTANEOUSLY CRIMPING AND  
REACTING DRAWN NYLON FIBERS WITH HOT  
ALCOHOLIC FORMALDEHYDE SOLUTION**  
Conrad Georg Baumann, Zurich, Switzerland, assignor  
to Heberlein Patent Corporation, New York, N.Y., a  
corporation of New York  
No Drawing. Filed Mar. 16, 1965, Ser. No. 440,323  
7 Claims. (Cl. 8—115.5)

This invention relates to a method for treating polyamide fabrics, and more specifically, it relates to a method for chemically crimping polyamides.

For purposes of this application the term "textile material" or "fabric" shall be understood to include fabrics and textile materials of all kinds, including fibers, filaments, yarns, threads, and any manner of knit or woven fabrics as well as non-woven or felted fabrics.

It is known that polyamide textile materials can be chemically crimped by the formation of asymmetrical, incomplete cross-linkings between amide groups of polyamide molecules. This cross-linking has been achieved by methoxylation of the polyamide, sulfonation of the methoxymethylate, and finally the formation of sulfide bonds between the molecules. Subsequently, the treated polyamide threads are subjected to a swelling treatment to at least double the volume of the original thread, and spontaneous crimping takes place. The treated fibers are then dried.

While the foregoing method is capable of producing certain interesting crimping effects, it has a number of serious disadvantages. It calls for three chemical reactions prior to the swelling treatment and requires relatively expensive sulfur compounds, such as thiourea. These sulfurous materials, moreover, not only produce disagreeable odors during processing but the odors are also difficult to remove from the treated fabric.

This invention provides a considerably simpler and cheaper process for obtaining crimping effects in polyamide materials. Such crimping is generally superior to the crimping effects obtainable by the prior art processes.

This invention also provides a novel chemically crimped polyamide material.

Briefly, the process of this invention spontaneously crimps and shrinks polyamide fabrics by treating them in alcoholic formaldehyde solutions in the presence of an acid catalyst at temperatures at least about 50° C. for times not significantly in excess of ten minutes. This process thus provides novel crimped polyamide fibers and filaments and provides fabrics having increased density with a softer, more desirable hand.

In practicing this invention it is necessary that the polyamide fibers or filaments be drawn prior to treatment with the alcoholic formaldehyde. It will be understood that a drawn polyamide fiber is one which has been placed under tension so as to increase its original length significantly. In practicing this invention the polyamide fibers should have been drawn to at least 250% of their original length, and they should preferably be drawn to 300% or more of their original length.

While the drawing of nylon *per se* does not form a part of this invention, it is hypothesized that such a drawing of the polyamide filaments orients the crystals or crystal-like structures in the fibers. In any event, if undrawn polyamide-containing fabrics are subjected to the treatment of this invention, the fibers have a tendency to become very stretchy and elastic and the desirable properties of crimped material are lost.

It is especially preferred to treat textile fabrics containing nylon 6, that is, polymers of  $\epsilon$ -aminocaproic acid.

In the process of this invention, it is believed that the

amide groups of the polymers are methoxylated. Contrary to the prior art processes, however, the crimping produced by this invention does not appear to be based on differential cross-linking, but rather appears to rise from substitution in the secondary amino group of the polyamides. Apparently, the number of sites for the formation of hydrogen bridges between adjacent molecules is reduced and the crystal structure or texture of the fiber-forming material is changed. This appears to be the cause of the crimping or shrinking.

Where yarns and threads are treated according to this invention, a strong crimping effect is obtained. Where woven and knit goods are treated, considerable shrinkage occurs and the density of the material is increased with consequent improvement of the hand. Moreover, when drawn polyamides are treated according to this invention the electrical conductivity of the fabric is enhanced and the propensity of the material to retain static electric charges is reduced. Not only are the hand and electric conductivity improved, but in addition the dyeability of the polyamide is enhanced. Moreover, the tearing strength of the polyamide filaments and fibers is surprisingly increased.

The treatment bath used in this process must furnish formaldehyde for interaction with the polyamide. Formaldehyde may be added directly to the alcoholic treatment bath or a substance producing formaldehyde under the reaction conditions can also be used in the bath. A preferred material for use in the treatment bath is paraformaldehyde.

The treatment bath should contain a relatively high concentration of formaldehyde. Generally, it is preferred that the bath contain at least about 75% by weight of formaldehyde, and the formaldehyde can be present in concentrations as high as the saturation point of the formaldehyde in the particular alcohol.

The formaldehyde is used in an alcoholic medium. The alcohols suitable for use in the practice of this invention are the lower aliphatic monohydroxy alcohols. Generally lower aliphatic alcohols containing from about 1 to about 6 carbon atoms are suitable. Preferred alcohols are methanol, ethanol, and isopropanol.

The temperature of the treatment should be at least about 50° C. in practicing this process. The upper temperature limit of the process is usually determined by the atmospheric boiling point of the alcohol used in the bath. With the readily available alcohols, it is preferred to carry out the process at temperatures in the range of from about 60° to about 80° C.

The time of treatment is very important in this process. While the treatment time will vary inversely as the temperature of the treatment, the time should be restricted to an upper limit of about 10 minutes. The use of a longer time will adversely affect the finished product, and some of the polyamide properties will be degraded by excessive treatment intervals. For example, treatment times on the order of 20 minutes result in partial fusion of the fabric and are very detrimental to the hand. Moreover, treatment of the fabric for as long as 20 minutes causes partial dissolution of the polyamide material and adversely affects the strength thereof. It has been found that a treatment of 5 minutes or somewhat less is generally adequate to produce the desired results. It is preferred in this process to treat the polyamide materials for a time on the order of from about 5 to about 10 minutes.

The treatment bath must also contain an acid catalyst. Suitable acid catalysts are ammonium bromide, calcium chloride, phosphoric acid, *p*-toluene sulfonic acid, mono-, di-, and trichloroacetic acid. Dicarboxylic acids such as

maleic acid are excellent catalysts. A preferred catalyst is oxalic acid.

After the treatment of the polyamide fabric has been carried out, the formaldehyde-containing solution should be removed from contact with the material. One of the most effective ways to remove the formaldehyde solution from the material is to wash it with an alcohol, conveniently the same alcohol used as the solvent in the solution, and then to wash all the alcohol out with cold water. After washing the treatment solution out of the material and drying, the material will then be suitable for further use or processing.

The following examples are given to illustrate some embodiments of this invention and not to indicate the entire scope of the invention, the scope being determined by the claims appended hereto.

*Example I*

A solution is prepared by dissolving 250 g. of paraformaldehyde (trioxymethylene) in 300 ml. of ethanol with vigorous stirring at a temperature of 65° C. After the formaldehyde is dissolved, 14.3 g. of anhydrous oxalic acid is added as a catalyst and the solution is filtered.

The temperature of the solution is raised to 80° C. and a skein of drawn nylon 6 yarn is immersed in the bath for 5 minutes to spontaneously crimp the yarn. Subsequently the yarn is thoroughly washed with ethanol, then with cold water, and dried.

This treatment results in a powerful crimping of the yarn and its tensile strength is found to be more than twice that of the original yarn.

*Example II*

The treatment solution is prepared by saturating 300 ml. of methanol with paraformaldehyde at a temperature of 65° C. and adding 15 g. of oxalic acid as a catalyst. The solution is then filtered.

Subsequently temperature is raised to 70° C. and a knitted fabric of nylon 6 yarn is immersed in the treatment bath for 10 minutes, washed thoroughly with alcohol and then with cold water, and dried.

The fabric is shrunken considerably in its dimensions and is found to have a soft, pleasant hand.

*Example III*

The treatment bath is prepared by saturating 300 ml. of isopropanol with formaldehyde at a temperature of 65° C. and subsequently adding 15 g. of oxalic acid as a catalyst. The solution is then filtered.

The bath is maintained at 65° C. and a woven fabric of drawn nylon 6 yarn is immersed in the bath for 10 minutes, washed thoroughly with ethanol and then with cold water, and dried.

After this treatment the fabric is considerably shrunken and exhibits an improved hand.

What is claimed is:

1. A process for crimping polyamide textile materials which comprises treating nylon textile fibers, which have been drawn to at least 250% of their original length and consisting essentially of a polymer of  $\epsilon$ -aminocaproic acid,

by immersing said fibers in a solution of at least 75% by weight of formaldehyde in a monohydric lower aliphatic alcohol containing an acid catalyst at a temperature of from at least about 50° C. to the temperature at which said alcohol boils at atmospheric pressure for a maximum of about 10 minutes, said time being inversely related to said temperature, until said fibers simultaneously shrink and become crimped.

2. A process for crimping polyamide textile materials which comprises treating nylon textile fibers, which have been drawn to at least 250% of their original length and consisting essentially of a polymer of  $\epsilon$ -aminocaproic acid, by immersing said fibers in a solution of at least 75% by weight of formaldehyde in a monohydric lower aliphatic alcohol containing an acid catalyst at a temperature of from at least about 50° C. to the temperature at which said alcohol boils at atmospheric pressure for a maximum of about 10 minutes, said time being inversely related to said temperature, until said fibers simultaneously shrink and become crimped, and subsequently washing the crimped nylon to remove the solution.

3. A process for crimping polyamide textile materials which comprises treating nylon textile fibers, which have been drawn to at least 250% of their original length and consisting essentially of a polymer of  $\epsilon$ -aminocaproic acid, by immersing said fibers in a solution of at least 75% by weight of formaldehyde in a monohydric lower aliphatic alcohol containing an acid catalyst at a temperature of from at least about 50° C. to the temperature at which said alcohol boils at atmospheric pressure for a maximum of about 10 minutes, said time being inversely related to said temperature, until said fibers simultaneously shrink and become crimped.

4. The process of claim 1 wherein the alcohol is selected from the group consisting of methanol, ethanol, and isopropanol.

5. The process of claim 1 wherein the catalyst is oxalic acid.

6. A process for crimping polyamide textile materials which comprises treating nylon textile fibers, which have been drawn to at least 250% of their original length and consisting essentially of a polymer of  $\epsilon$ -aminocaproic acid, by immersing said fibers in a solution of at least 75% by weight of formaldehyde in a monohydric lower aliphatic alcohol containing an acid catalyst at a temperature of from about 60 to about 80° C. for from about 5 to about 10 minutes, said time being inversely related to said temperature, until said fibers simultaneously shrink and become crimped.

7. A crimped polyamide textile material prepared according to the process of claim 1.

**References Cited**

**UNITED STATES PATENTS**

2,441,085 4/1948 Schneider ----- 8—115.5

NORMAN G. TORCHIN, *Primary Examiner*.

H. WOLMAN, *Assistant Examiner*.